

Patented Aug. 20, 1929.

1,725,445

# UNITED STATES PATENT OFFICE.

VICTOR D. DAVIGNON, OF ATTLEBORO, MASSACHUSETTS, ASSIGNOR TO GENERAL PLATE COMPANY, OF ATTLEBORO, MASSACHUSETTS, A CORPORATION OF RHODE ISLAND.

## PRECIOUS-METAL PLATE.

No Drawing.

Application filed May 3, 1926. Serial No. 106,556.

This invention relates to plated metal and methods of producing the same, and particularly concerns an improvement in plated products which comprises a backing of relatively cheap low specific gravity metal surfaced with a comparatively thin layer of precious metal.

Heretofore in producing precious metal plate such as gold or silver plate it has been common to use as the backing a malleable alloy of copper containing zinc and tin, which alloy although otherwise suitable for forming the product possesses the disadvantage of a relatively high specific gravity, and it is among the objects of my invention to produce gold or other plate in which the base metal or backing has relatively low specific gravity.

As an example of a suitable backing for plate made according to my invention I may use an alloy containing aluminum for securing a low specific gravity. So that this alloy may be worked by mill processes of alternate mechanical attenuation and annealing the constituents of this alloy and their relative proportions preferably are such that the alloy is sufficiently malleable or ductile when cold to permit attenuation by the usual mill operation of rolling or drawing and to permit annealing after the alloy has been hardened as a result of the attenuating operation.

As satisfactory for aluminum alloy for economic use in producing gold plate by alternate rolling and annealing I have found that the alloy may be compounded so as to contain from about 2 to 10 percent by weight of aluminum and a material proportion of copper. Preferably copper is the only metal other than aluminum present in substantial amount, but if desired small amounts of other metals such as zinc, tin, nickel, etc. commonly employed for imparting special properties may be incorporated. This alloy is of materially lower specific gravity than that heretofore used in connection with the production of precious metal plate and is malleable when cold, while by a process hereinafter described it may be annealed to permit production of plate by machinery commonly employed in the art for this purpose. If the aluminum content exceeds 10 percent by weight of the alloy the latter may be economically rolled only when hot, which, if the precious metal used is a gold

alloy containing a substantial proportion of gold, renders the alloy impractical for use in production of gold plate because the gold alloy can satisfactorily be rolled by usual mill machinery only when cold.

As an example of the improved process of producing plate, but without limitation thereto, I may form the backing from a plate of alloy containing by weight 92 percent copper and 8 percent aluminum, said plate being about three-quarters of an inch thick, 3 inches wide, and 14 inches long. On one or both sides of the plate I now place a sheet of solder, as for example silver solder about .003 of an inch thick, and on this sheet place a sheet of gold alloy, as for example 14 carat copper-gold alloy, the thickness of the gold alloy sheet being such that its weight is from one-half to one-four hundredth of the weight of the backing. The built up plate of base metal, gold alloy, and solder I place in a soldering furnace and after heating to the soldering temperature subject it to a pressure of about 5 tons, which with use of suitable flux as herein-after described effects soldering of the gold alloy to the backing. After the soldering operation the billet is allowed to cool and then is passed between the rolls of a mill to reduce its thickness, the rolling operation being repeated with successive reduction in thickness of the material until the material reaches a degree of hardness necessitating annealing before it may be further reduced. The material is then annealed by a process hereinafter described and the rolling operation repeated. By alternately subjecting the material to the rolling and annealing operations it is finally reduced to the required thickness.

In order to make a homogeneous union by the soldering operation between the gold alloy sheet and the aluminum alloy backing I have found it desirable to eliminate aluminum oxide or other aluminum compounds which interfere with the soldering operation, and for this purpose I place on the sheet of silver solder or on the faces of the backing and gold alloy in contact with the silver solder suitable flux, having found satisfactory for this purpose potassium bifluoride, calcium chloride, a mixture of one part calcium chloride and two parts potassium bifluoride, cryolite, and sodium fluoride, these substances preferably being mixed with

borax. As examples of fluxes, but without limitation thereto, I may use a mixture consisting of one-half borax and one-half cryolite, or two-thirds borax and one-third sodium fluoride. Conveniently the flux may be applied in the form of an aqueous solution in which the parts may be dipped, or the parts may be sprayed with the solution, or I may apply the flux in the form of a powder, 10 say with a brush or puff. It will be noted in the examples given that the materials mixed with the borax are all halogen salts of alkaline earths.

As hereinbefore explained, economically 15 to attenuate the billet in the mill it must ordinarily be annealed after the attenuating operation has progressed to such extent that the partially reduced billet becomes hard. As an example of a satisfactory annealing 20 operation, but without limitation thereto, I may heat-treat the material by raising it to a temperature of from about 900 to 1300 degrees Fahrenheit in an annealing furnace and suddenly plunge it while at that temperature 25 into a quenching liquid, as for example water at room temperature, which will render both the gold alloy and aluminum alloy backing sufficiently malleable or ductile for continuation of the attenuating operation.

I have also found as suitable for alloy, especially where wear resisting qualities are desired, that some of the aluminum in the 30 above example may be substituted by iron or manganese. As an example of such alloy, but without limitation thereto, it may consist of about 6.5 percent by weight of aluminum, about 1 percent by weight of either iron or manganese, with the remainder copper.

As a substitute for aluminum I have found suitable a mixture of silicon and manganese, the latter being sufficient in amount 40 to counteract the hardening effect of the silicon. As an example of such alloy, but without limitation thereto, it may consist of about 4 to 4.5 percent silicon and about 1 percent manganese with the remainder copper.

My improvement is distinguished from prior processes and products in that I employ as a backing a cold-malleable, copper alloy containing sufficient aluminum or like 50 low specific gravity metal, such as silicon, materially to reduce its specific gravity, a homogeneous union being effected between the backing and the precious metal, and the product being heat treated between the attenuating operations to render it ductile or malleable. In the preferred example the 55 backing contains from about 2 to 10 percent of aluminum, 8 percent being satisfactory, and the union between the backing and precious metal is effected by soldering in the presence of a flux eliminating the deleterious 60

effect of aluminum oxide on the soldering, while annealing is effected by heat treatment comprising heating the billet and plunging it into cold quenching liquid while at a temperature of about 1000 degrees Fahrenheit. 70

It will be understood that wide deviations may be made from the examples of the invention herein described without departing from the spirit of the invention.

Claims—

1. That method of producing a plated product consisting of a layer of gold alloy on a backing of copper-aluminum alloy, the latter containing sufficient aluminum materially to reduce its specific gravity but not more than about 10 percent by weight, and being sufficiently malleable to permit substantial attenuation thereof by rolling or drawing while cold, which comprises effecting a homogeneous union of relatively thick pieces 80 of said gold alloy and backing, and attenuating the united materials by repeated rolling or drawing thereof while cold.

2. That method of producing a plated product consisting of a layer of gold alloy on a backing of copper-aluminum alloy, the latter containing sufficient aluminum materially to reduce its specific gravity but not more than about 10 percent by weight, and being sufficiently malleable to permit substantial 90 attenuation thereof by rolling or drawing while cold, which comprises effecting a homogeneous union of relatively thick pieces 95 of said gold alloy and backing; attenuating the united materials by repeated rolling or drawing thereof while cold, with heat treatment 100 between rolling or drawing operations for annealing the backing after the same has been hardened by said operations.

3. That method of producing a plated 105 product consisting of a layer of gold alloy on a backing of copper-aluminum alloy, the latter containing sufficient aluminum materially to reduce its specific gravity but not more than about 10 percent by weight, and being sufficiently malleable to permit substantial 110 attenuation thereof by rolling or drawing while cold, which comprises effecting a homogeneous union of relatively thick pieces 115 of said gold alloy and backing by soldering one to the other in the presence of a flux capable of effecting soldering and eliminating the deleterious effects of aluminum oxide, and attenuating the united materials 120 by repeated rolling or drawing thereof while cold.

4. That method of producing a plated product consisting of a layer of gold alloy on a backing of copper-aluminum alloy, the latter containing sufficient aluminum materially to reduce its specific gravity but not more than about 10 percent by weight, and being sufficiently malleable to permit substantial 125 attenuation thereof by rolling or drawing while cold, which comprises effect- 130

ing a homogeneous union of relatively thick pieces of said gold alloy and backing by soldering one to the other in the presence of a flux capable of effecting soldering and containing a halogen salt of an alkaline earth, and attenuating the united materials by repeated rolling or drawing thereof while cold.

5. That method of producing a plated product consisting of a layer of gold alloy on a backing of copper-aluminum alloy, the latter containing sufficient aluminum materially to reduce its specific gravity but not more than about 10 percent by weight, and 10 being sufficiently malleable to permit substantial attenuation thereof by rolling or drawing while cold, which comprises effecting a homogeneous union of relatively thick pieces of said gold alloy and backing by 15 soldering one to the other in the presence of a flux capable of effecting soldering and containing borax mixed with a halogen salt of an alkaline earth, and attenuating the united materials by repeated rolling or drawing 20 thereof while cold.

6. That method of producing a plated product consisting of a layer of gold alloy on a backing of copper-aluminum alloy, the latter containing sufficient aluminum materially to reduce its specific gravity but not more than about 10 percent by weight, and 30 being sufficiently malleable to permit substantial attenuation thereof by rolling or drawing while cold, which comprises effecting a homogeneous union of relatively thick pieces of said gold alloy and backing; attenuating the united materials by repeatedly 35 rolling or drawing them while cold, and between rolling or drawing operations, after 40 the backing has been hardened thereby, heating said materials and quenching them at such temperatures as will render the backing sufficiently malleable for said operations to be continued.

45 7. That method of producing a plated product consisting of a layer of gold alloy on a backing of copper-aluminum alloy, the latter containing sufficient aluminum materially to reduce its specific gravity but not more than about 10 percent by weight, and 50 being sufficiently malleable to permit substantial attenuation thereof by rolling or drawing while cold, which comprises effecting a homogeneous union of relatively thick pieces of said gold alloy and backing; attenuating the united materials by repeatedly 55 rolling or drawing them while cold; and between rolling or drawing operations, after 60 the backing has been hardened thereby, annealing said backing by heating said materials and plunging them, while at a temperature of about 1000 degrees Fahrenheit, into cold quenching liquid, to permit said operations to be continued.

65 8. That method of producing a plated

product consisting of a layer of gold alloy on a backing of copper-aluminum alloy, the latter containing by weight not more than about 10% of aluminum but enough materially to reduce its specific gravity and being sufficiently malleable to permit substantial attenuation thereof by rolling or drawing while cold, which comprises effecting by soldering a substantially homogeneous union 70 between relatively thick pieces of said gold alloy and backing; and attenuating the united materials by rolling or drawing thereof while cold, with heat treatment thereof between the rolling or drawing operations for annealing the backing after the 75 same has been hardened by said operations.

9. That method of producing a plated product consisting of a layer of gold alloy on a backing of copper-aluminum alloy, the latter containing by weight not more than about 10% of aluminum but enough materially to reduce its specific gravity and being sufficiently malleable to permit substantial attenuation thereof by rolling or drawing while cold, which comprises placing 80 between relatively thick pieces of said gold alloy and backing a thin sheet of silver solder and a soldering flux, the latter containing borax and a halogen salt of an alkaline earth, effecting homogeneous soldering 85 of said pieces by forcing one toward the other with great pressure while at high temperature, attenuating the united materials by repeatedly rolling them while cold; and between rolling or drawing operations, after 90 said backing has been hardened thereby, annealing the backing sufficiently to permit said rolling or drawing operations to be continued, said annealing comprising heating said materials and while at about 1000 95 degrees Fahrenheit quickly quenching them with water at about room temperature.

10. Plated products comprising a layer of gold alloy containing a material amount of gold on a backing of copper-aluminum alloy, 110 the latter capable of being attenuated by rolling or drawing while cold and containing a material proportion of copper and from about 2 to 10 percent by weight of aluminum.

11. Plated products comprising a layer of gold alloy containing a material amount of gold on a backing of copper-aluminum alloy, the latter capable of being attenuated by rolling or drawing while cold and containing a material proportion of copper and about 8 per cent by weight of aluminum.

12. Plated products comprising a layer of gold alloy containing a material amount of gold on a backing which can be attenuated 115 by rolling or drawing while cold and consisting of about 8 percent by weight of aluminum and about 92 percent by weight of copper.

13. A plated product comprising a layer 130

- of gold alloy on a backing of copper alloy, the gold alloy containing at least 25 percent by weight of gold, the base metal content of the copper alloy having sufficient aluminum materially to reduce the specific gravity of said alloy, said copper alloy having sufficient copper relative to the base metal content to render the alloy capable of being attenuated by rolling or drawing while cold, 10 the aluminum content of said copper alloy being in all cases at least 2 percent by weight, and, when the said copper alloy is exclusively copper and aluminum, the aluminum content not exceeding 10 percent by 15 weight.
14. A plated product comprising a layer of gold alloy on a backing of copper alloy, the gold alloy containing at least 25 percent by weight of gold, the copper alloy being 20 predominantly copper and containing sufficient aluminum materially to reduce its specific gravity but not enough aluminum to prevent it from being attenuated by rolling or drawing while cold, the aluminum content 25 of said copper alloy being in all cases at least 2 percent by weight, and, when the said copper alloy is exclusively copper and aluminum, the aluminum content not exceeding 10 percent by weight.
- 30 15. A plated product comprising a layer of gold alloy containing a material amount of gold on a backing which can be attenuated by rolling or drawing while cold and consisting of from about 2 to 10 percent by weight of aluminum with the remainder 35 copper.
16. A plated product comprising a layer of 14 carat gold on a backing of copper-aluminum alloy which can be attenuated by rolling or drawing while cold and containing about 92 percent of copper and about 8 percent of aluminum. 40
17. Plated products comprising a layer of gold alloy containing at least 25% by weight of gold on a backing of copper alloy, the latter capable of being attenuated by rolling or drawing while cold and containing a material proportion of copper and from about 2 to 10% by weight of aluminum. 45
18. A plated product comprising a layer of 14 carat gold on a backing of copper alloy, the latter capable of being attenuated by rolling or drawing while cold and containing a material proportion of copper and sufficient aluminum materially to reduce its specific gravity but not more than about 10 percent by weight of aluminum. 50 55

In testimony whereof, I have signed my name to this specification.

V. D. DAVIGNON.